# EUROPEAN PATENT APPLICATION

(11) **EP 0 099 137 A1**
(43) Date of publication of application: **25.01.1984**
(21) Application number: 83200678.7
(22) Date of filing: 11.05.1983
(51) Int. Cl.: F16F 15/00, C22C 9/04

(54) **Vibration absorbing article made of shape memory alloy**

(30) Priority: 13.05.1982 NL 8201985
(71) Applicant: Leuven Research & Development V.Z.W., B-3000 Leuven (BE)
(72) Inventor: Delaey, Luc, B-3060 Bertem (BE); Van Humbeeck, Jan, B-3030 Heverlee (BE)
(74) Representative: Ryckeboer, Leo L.H.

(57) **Abstract**

The invention relates to an article with vibration damping capacity and includes a metal alloy with potential shape memory properties whereby the alloy is in the martensitic state at room temperature or above and absorbs in this state in a durable way at least 10 percent of the imposed vibration energy with a vibration amplitude greater than 10-⁵ and smaller than the limit of microplastic. deformation.

## Description

The invention relates to an article suitable for damping mechanical vibrations and composed of a metallic alloy with potential shape memory properties, which article- is in the martensitic state particularly at ambient temperature.

Metallic alloys with shape memory characteristics can, with more or less success and owing to internal friction in the martensitic state, convert the energy of deformation by vibrations into heat. This capacity mainly occurs in the martensitic state so that these metals belongg to the group of hidamets: However, the damping capacity of memory alloys is not in all circumstances sufficiently .high or stable enough in time or after a number of-vibrations ; for example they may lose their damping capacity relatively quickly.

Shape memory alloys are known to be characterized by a transformation from the martensitic state at lower temperature to an intermetallic compound in the β-phase. This may go together with a macroscopic change in the shape of the article which takes place in the reverse direction when cooled again to the martensitic phase.

The characteristic transformation temperatures are A ₛ and A_{f} during heating and Mₛ and M_{f} during cooling. Mechanical loading has an influence on these temperatures. It is an object of the invention to dampen, in particular at room temperature, a greater share of the vibration energy absorbed by an article with potential shape memory properties and so to transform its energy into another form of energy and to optimize the amount and durability of the damping action after repeated vibration loading. Repeated vibration loading refers to those circumstances whereby the article goes through an unlimited number of vibration cycles in the form of, for example, a standing wave vibration or repeated impact loading within a given period of time, for example a number of shocks per minute or per hour.

The article according to the invention thus essentially comprises an alloy with potential shape memory characteristics which at ambient or higher temperature is entirely in the martensitic state and which in this condition absorbs in a durable way at least 10% of the imposed vibration energy with a vibration energy with a vibration amplitude superior to 10 and which is preferably below the limit of microplastic deformation. This limit is usually considered to be at 10 . Preferably the range between 10⁻⁴ and 10 ⁻³ is used. The vibration amplitude is here defined as a dimensionless magnitude of deformation : 10⁻³ means 0.1% deformation measured between the neutral position and the maximum deviation.

To render an article made of an alloy with shape memory capacity entirely martensitic it must, after the structure has been betatized, be cooled down in the prescribed manner to above Mₛ, and, after a possible treatment time at this temperature, be cooled down, within certain limits of cooling speed, to below the M_{f} temperature.

To obtain an improved damping capacity the article in the martensitic state must not be submitted to noteworthy deformation and must, when used as a vibration dampener, stay entirely in this state. This means that there must be no deposits from other phases, and, after the article has been cooled to below M_{f2} there may at no moment be a formation of another phase, neither through temporary heating above- Aₛ, nor owing to deformation or stresses. This temperature Aₛ must therefore be higher than the temperature at which the vibration is imposed, and practically always above room temperature.

The difference between A and vibration temperature, however, may vary between 1°C and 100°C or higher. The damping level may decrease accordingly as this difference becomes greater.

For achieving a durable damping capacity the thermal prehistory of the alloy is particularly important, i.e. the manner of cooling the alloy down from the higher temperature to which it was heated to bring it entirely in the 3-phase-. The damping level also depends upon the alloy composition. According to the invention an article made of shape memory alloy is preferably brought to the equilibrium temperature of the (stable) β-phase and cooled down in a quenching medium to a temperature above Mₛ, for example- to a temperature between 70°C and 200°C (if M ₛ is at room temperature), and it is kept at this temperature for a period of time (a t) which may vary from one minute to a few hours, for example thre hours. The selected time will be longer when the treatment takes place close to M (M at relatively low temperature) or when the quenching speed is higher. The time is shorter when the treatment takes place at a temperature significantly higher than M ₛ or when the cooling speed is smaller. This treatment may for example take place in hot oil between 70°C and 100°C or 200°C when M is between 30°C s and 50"C.

The time a t is not arbitrarily long because precipitation of some elements in, for example, bainite or δ -phase (a metallic solution) must be avoided because this may adversely influence the damping capacity. The alloy must consist of a metastable β-compound with mainly substitutionally dissolved subsidiary elements and must, when further cooled down below M and M_{f}, be fully transformed into martensite at a cooling rate preferably between 0.5°C and 10°C per minute. The time a t depends upon the absolute temperature at which the treatment is conducted and upon the composition and is optimized for each individual case.

In addition or as an alternative, improved damping characteristics are obtained by the judicious selection of the alloy composition.

The heat treatment (a t) must then be adapted to the thermo-mechanical history of the alloy.

The ambient temperature at which the vibration damping according to the invention is applied is in most cases between 0°C and 40°C, i.e. at room temperature. The A ₛ temperature of undeformed martensite must then be higher than 40°C. If for any reason a partial transformation to austenite has occurred, this must be neutralized by cooling again below M_{f}.

Although the articles according to the- invention can be used as such as construction materials, they will usually be fixed to components of fixed constructions. A fixed construction is any mechanical construction whereby during use one or more elements are submitted to mechanical vibration, either continuously or intermittently. This may, for example, occur during the impact on the matrix of a forming press, a part of a machine tool, on the protective plate of a rotating cabling machine or motor, parts of a moving vehicle of metal, plastic or composites. However, the natural damping which takes place in plastics or composites is usually greater than that of hidamets. The articles of shape memory alloys can be fixed to the construction of solid material as a functional component or as a non-functional component, for example as a glued plate, profile, rod, connecting element, impact cushion, ballast weight, etc. The shape of the object and its location are preferably obtained according to known techniques so that all vibrations and in particular low frequency sound vibrations, for example below 100 Hz, are dampened ; such vibrations are very penetrating and annoying. The prevailing vibration frequency is also governed by the vibration source and the natural-frequency of the system. However, the occurring frequency is of. secondary importance to the damping itself. It is also possible that the damping component is a combination of an article of shape memory alloy and a thermo-hardening or thermo-plastic material, an elastomer, or a combination of these materials.

The damping is quantitatively expressed as the loss factor Q (or η). The loss factor is the ratio of the energy fraction ΔW per unit of volume of the article which during vibration is lost through internal friction to the total energy content W in the form of vibration generated per unit of volume multiplied by 2 Π :

The loss factor can be determined at various temperatures with a type DMA 980 and 981 device, "Dynamic Mechanical Analyzer", distributed by Du Pont Instruments, Wilmington DE 19898 - USA with the adjoined description E 16368. The samples which are tested at their natural frequences in the following examples are usually plates made of shape memory alloy with a length of approximately 30.5 mm, a width of 5 to 10 mm, and a thickness of 0.3 _{L}o 1.5 mm. The frequency possible in this setup is between 3 Hz and 100 Hz, but is usually comprised between 20 and 50 Hz. By avoiding a deformed condition in the martensitic state, the shape memory of the alloy is not directly used.

Most shape memory alloys are suitable for vibration damping, but more readily available materials such as copper alloys and more particularly Cu-Zn-Al-containing alloys are preferred. In some cases Cu is to some extent substituted by one or more elements such as for example Ni. Cu-Al-Ni, Cu-Sn, Ni-Ti and other compounds may be considered for the same application, but this list is certainly not exhaustive.

The alloy composition changes the A ₛ transition temperature so that a selection of the composition can be made in respect of the required circumstances (temperature) at which the vibration is applied. By the combination of a thermo-mechanical pretreatment and a selected composition, the working range and durability of the vibration damping can be fixed on the basis of a vibration analysis test. It is assumed that the loss factor Q⁻¹ after 100.000 vibration cycles should be higher than 2X, in some cases this limit should be 4% even after 1.000.000 cycles. In other circumstances the limit will be for example 10.000 cycles. This damping stability may be improved by adapting the treatment time a t in the β-phase or by using another composition for the alloy or by the combination of both. The applied vibration frequency for which the specific damping capacity (ΔW/W) is at least 10% refers, according to the invention preferably, to the low frequency range below 100 Hz.

The invention will now be clarified by means of some graphs. The alloy composition is always indicated in percent by weight.
Figure 1 shows. the change of the loss factor at decreasing temperature ;
Figure 2 shows the variation of the loss factor with the number of cycles ;
Figure 3 shows an example of heat treatment applied to the alloy ;
Figure 4 shows a detail of the ternary Cu-Zn-Al diagramme ;
Figure 5 shows the influence of Ni substitution in Cu-Zn-Al on the stability of the loss factor ;
Figure 6 shows a damping curve in time for various amplitudes.

The damping trend according to Figure 1 was determined by means of the aforementioned D.M.A. damping analyzer. A metal plate of shape memory alloy was made to vibrate at its natural frequency. As from a temperature in the metastable β-phase it was gradually cooled down whereby the loss factor Q was determined ; its trend is shown by curve 1. When crossing Mₛ in zone 2, Q⁻¹ rises very rapidly to a maximum 3 to drop again so that the curve 1 shows a bending point 4 in the vicinity of M_{f}. Then the curve shows a minimum 5 to reach after the rise in point 6, a second maximum 7 to diminish gradually in section 8. At room temperature K there is substantially stable damping and this corresponds with the zone 6. When heating again an analogous 1' curve is registered whereby the A may be situated near M ₛ without that there is a direct relationship. The maximum of the loss factor then occurs between A and A_{f}.

However, the loss factor Q established in this manner is but a series of momentary recordings at a number of temperatures. If, for example, the temperature in the transition area between Mₛ and M_{f} is kept constant then the loss factor drops after a few vibration cycles to a small residual value. The behaviour shown in Figure-1 is a typical example for a given vibration amplitude. For a substantially higher vibration amplitude the damping will remain substantially on the maximum level when the temperature drops below M_{f}.

### Example 1

Figure 2 shows the results of the damping measurement with the so called D.M.A. device or an alloy (curve 10) at a peak amplitude of 0.2 mm. The dimensions of the sample plates were 31 x 7 x 1 mm. The sample was composed of 73.7 % Cu, 20.3 % Zn and 6 % Al (see alloy h in table II hereafter) with a grain size of approximately 0.5 mm to 1 mm and was maintained at 95°C after betatizing at 750°C for 15 minutes and after quenching to above M ₛ for 30 minutes. The sample was further cooled in the air and tested for damping behaviour at 22°C. The initial value of the damping factor is . After an initial damping maximum after 3.6 kS (kiloseconds) in point 11 (Q⁻¹≃ 5,5 x 10⁻²) the loss factor gradually decreases to 0.9 at approximately 11 kS. At that moment the amplitude 1 is brought to 0.8 mm for 2 seconds after which a new damping characteristic 12 analogous to the first 10 is generated. This mechanical regeneration of the damping is also- possible by a mechanical relaxation (releasing) of the sample. The line 13 shows a simultaneous registration of the frequency which fluctuates between 25 en 30 Hz. The curve 14 shows the damping trend of an identical sample in the same vibration test. However, this sample was directly quenched to martensite in water of 20°C. If the martensitic trans- formation is not achieved entirely, the damping will become negligible almost immediately as shown by curve 15. Other compositions having damping capacities are shown in table II.

Figure 3 shows the course of the thermal treatment as a function of time and versus the transformation temperatures Mₛ, M_{f} during cooling and Aₛ, A_{f} during heating to obtain an improved damping effect, whereby further the loss factor in time stays above a limit value for a longer period. The line 16 shows the'change of temperature with the time t. The hatched areas A, B and C indicate when insufficient damping occurs. Thus quenching to below M_{f} without heat treatment (a t) places the damping capacity in the unfavourable area A. When, on the other hand, (after maintaining under M ) the temperature is allowed to rise above A ₛ (so that again a transformation to austenite takes place) the damping results will worsen again at these temperatures in the vibration test (area B). Therefore it will be necessary to apply a thermal regeneration in the form of a renewed thermal treatment a t after which further cooling down to under M_{f} is carried out to get out of this unfavourable area B at its right side (see drawing). Damping will stay low in any vibration test above A : this is suggested by area C.

### Example

An alloy consisting of 75.57 % Cu, 14.06 % Zn, 8.17 % Al and 2.03 % Ni (percent by weight - alloy g in table I) was, after being quenched from the β-zone to 70°C, kept at this temperature for a period (a t) of 120 min. The alloy was subsequently cooled down in water ice. Then the sample was heated again to 20°C, the testing temperature, below A . The damping trend is reflected by curve 10 in Figure in a vibration test as described in example 1. In other words, the damping starting level 11 (after a vibration period of 3 kS) is clearly raised versus the value and the damping drop in time is low.

### Example 3

Figure 4 shows a ternary diagram with a number of compositions of Cu-Zn-Al alloys to which the invention can be applied. The important zone is located between the points 17, 18, 19 and 20. The following points 17 : 1 % Al and 35 % Zn ; 18 : 5 % Al and 21 % Zn ; 19 : 12.5 % Al and 0 % Zn ; 20 : 14 % Al and 0 % Zn, all in percent by weight, the remainder each time mainly Cu, possibly replaced by a few percent of another metal, for example Ni up to 2.3 %. The transformation temperature M ₛ lies between approximately 0°C and 200°C. The difference between A and M is a few °C. The actually measured transformation temperature is a more efficient criterion than the composition which is only a target parameter because of the accuracy limits of the analysis. The alloys in table I and II belong to this zone.

### Example 4

Figure 5 shows the influence of the composition of such alloys on the damping factor. Ni is added in weight as a substitution of Cu because only a small deviation of Mₛ is expected at the same Al - Zn proportion. The compositions of the examined alloys c, e, f and g as well as their Aₛ and Mₛ temperatures are shown in table I. The line 21 is the damping factor after 100.000 vibration cycles, the line 22 after 200.000 cycles and the line 23 after 300.000 cycles. The substitution of 2 % Cu by 2 % Ni has a stabilizing effect on the value of the damping factor. The treatment time a t was one hour at 120°C each time. It is evident that a comparable behaviour can be found, particularly with copper alloys where a transition from a p Hume-Rothery metallic compound towards a martensitic state at suitable temperature is possible.

However, the treatment time a t may be decisive for a positive or negative result. So the damping factor, inter alia in example 4 and for an alloy "a" was significantly smaller when. the time a t was reduced from 1 hour to either 30 minutes or 15 minutes.

### Example 5

Figure 6 relates to an alloy f in table I and shows the influence of the amplitude on the loss factor for vibrations during a longer time (kilo seconds). The figures next to the different curves are the vibration amplitudes imposed. At lower amplitude the damping factor is variable in time, whereas at higher amplitudes around 10⁻³ the damping factor stays practically equal or even at an increased level for a longer time. The natural frequency of the sample usually lies around 25 and 30 Hz. When the alloys have a fine grain then the damping characteristics are often slightly less favourable.

## Claims

1. An article with vibration damping capacity comprising a metal alloy with potential shape memory properties characterized in that the alloy is in the martensitic state at room temperature or above and absorbs in this state in a durable way at least 10 % of the imposed vibration energy with a vibration amplitude greater than 10-5 and smaller than the limit of microplastic deformation.

2. An article according to claim 1 characterized in that the vibration amplitude is greater than 10-4.

3. An article according to claim 1 or 2 characterized in that the vibration amplitude is smaller than 10-3.

4. An article according to claims 1 or 2, characterized in that the article is obtained by quenching the alloy from a temperature where it comprises a stable beta-phase up to a temperature above its M , after which it is maintained at this temperature for an adapted period of time and next cooled to below a temperature M_{f}.

5. An article according to one of the foregoing claims characterized in that the metal alloy comprises more than 50 % Cu.

6. An article according to claim 5 characterized in that it possesses a composition within the area bounded by points 17, 18, 19, 20 in Figure 4.

7. An article according to claim 6 characterized in that in this alloy 1 % to 2.3 % by weight of Cu is substituted by Ni.

8. A solid structure characterized in that at least one article according to claim 1 or 2 is fixed to it for damping the mechanical vibrations generated in it and having an amplitude greater than 10-5 and smaller than the microplastic deformation of the article.
